

# UNITED STATES PATENT OFFICE.

JAS. S. SUTER AND GEO. M. PALMER, OF BALTIMORE, MARYLAND.

## IMPROVEMENT IN WRAPPERS FOR CIGARS.

Specification forming part of Letters Patent No. 21,704, dated October 5, 1858.

*To all whom it may concern:*

Be it known that we, JAMES S. SUTER and GEORGE M. PALMER, of Baltimore, in the county of Baltimore, in the State of Maryland, have invented a new and Improved Mode of Manufacturing Wrappers for Cigars and Chewing-Tobacco; and we do hereby declare that the following is a full and exact description thereof.

Our invention consists in taking pearlash, powdered sal-ammoniac, lobelia or Indian tobacco, oil of anise-seed, oil of caraway, alcohol, rum, grass rope, cascara bark, opium, sumac, and with stems or refuse tobacco manufacturing sheets for various purposes—namely, wrappers for cigars or tobacco and sheets for wrapping woolen goods to prevent moths from cutting them, lining for boxes for same, and covering for carpets, the article made in this way being preferable to the natural tobacco, first, because it can be made of any required length or breadth; secondly, by this process the oil that the tobacco contains, so deleterious to health, is destroyed; and, thirdly, that woolens of all kinds can be wrapped in it, as the sheets can be made of any required length, breadth, or thickness.

To enable others skilled in the art to make and use our invention, we will proceed to describe its construction and operation.

Take eight pounds of pearlash, three pounds of powdered sal-ammoniac, one pound of lobelia or Indian tobacco, fifty pounds of sumac-leaves, five pounds of grass rope, the rope to

be previously boiled in lime-water, one-quarter pound oil of anise-seed, one-quarter pound oil of caraway, one-quarter pound cascara bark, mixed with one-half gallon of alcohol, three gallons New England rum, with stems or scraps of tobacco first softened with water. Beat the whole into a fibrous pulp, and sheet out on the same machinery as is used for sheeting paper, regulating the same so as to make it thick or thin, according to the purpose for which it is used.

Being aware that the stems and refuse tobacco have been before used for making a material similar to paper and for like purposes by John Adcock, in England, we desire to disclaim the use of said stems and refuse tobacco; but

What we claim as our invention, and desire to secure by Letters Patent, is—

Taking pearlash, powdered sal-ammoniac, lobelia or Indian tobacco, oil of anise-seed, oil of caraway, alcohol, grass rope, rum, cascara bark, opium, sumac, and stems or refuse tobacco, and converting it into sheets for wrapping woolen goods to prevent moths from cutting them, lining for cases for the same, covering for carpets, and wrappers for cigars or tobacco.

JAS. S. SUTER.  
GEORGE M. PALMER.

Witnesses:

E. R. BAXTER,  
Wm. M. RINLE.